

Nov. 20, 1934.

R. H. ATKINSON

1,981,715

ELECTRODEPOSITION OF METALS

Filed July 9, 1932



INVENTOR.

Ralph Hall Atkinson,

BY

Byrnes, Stellins, Parmelee + Blenko

ATTORNEYS.

## UNITED STATES PATENT OFFICE

1,981,715

## ELECTRODEPOSITION OF METALS

Ralph Hall Atkinson, Acton, England, assignor  
to The International Nickel Company, Inc.,  
New York, N. Y., a corporation of Delaware

Application July 9, 1932, Serial No. 621,619  
In Great Britain July 11, 1931

3 Claims. (Cl. 204—1)

This invention relates primarily to electroplating and the electro-deposition of metals and alloys.

It is an object of the invention to provide a bath which shall have a long life without the use of a soluble anode.

Other objects and advantages will become apparent from the following description.

The invention consists essentially in the use of 10 an insoluble anode in a diaphragm cell with an ammoniacal anolyte substantially free from any metal compound and with a catholyte which comprises an ammoniacal solution of a compound or compounds of a metal or metals and which is 15 capable of yielding electro-deposits.

The commercial development of ammoniacal electrolytes has not received much attention because previously baths of this type could have only a short life on account of the fact that most 20 metal anodes are insoluble in these electrolytes, with the consequence that the metal content of the latter had to be maintained by periodical additions of salts thereby leading to undesirable accumulation of acid radicals in the plating solution, so that although in certain cases the presence 25 of the diaphragm may not affect the nature of the deposit, e. g. copper and nickel, it has the advantage that it enables the electrolyte, suitably replenished from time to time, to be used for 30 a very much longer time than would be possible without a diaphragm.

The invention is particularly applicable to palladium and alloys thereof, although it is in no way limited to these. It is, therefore, most convenient 35 first to describe the application of the invention to the deposition of palladium and then to indicate some further applications.

It is known to use for plating purposes a solution 40 of palladosammine chloride (dichloro-diaminopalladium) in ammonia in an ordinary electrolytic cell, but although the initial deposits may be good the deposits are unsatisfactory after a short time. In proceeding in accordance with the present invention, however, the catholyte 45 consists of a solution in ammonia of a palladium-ammino compound such as palladosammine chloride. The deposits produced are then found to be consistently good.

The improved results are believed to be mainly 50 due to the fact that when the palladium tetrarammine cation, which is present in an ammoniacal solution of palladosammine chloride, decomposes into palladium and ammonia, the latter reacts at the anode with chlorine to form ammonium chloride which accumulates undesirably

in a non-diaphragm cell, but which in a diaphragm cell, according to the invention, is formed only in the anolyte where its accumulation does not affect the plating process because part of the anolyte can be evacuated periodically. The palladium on the other hand, being wholly cationic, migrates to the cathode and thus can easily be kept within the catholyte compartment. However, the invention is not dependent on the accuracy of the above theory. 60 65

The evacuation of part of the anolyte can be effected in any convenient way either continuously or periodically. The anolyte removed may be replaced either by water or by ammonia solution. 70

In carrying out the process with palladosammine chloride the catholyte may conveniently consist of an aqueous solution containing about 5 grams of free ammonia and about 20 grams of palladium per liter. The anolyte may consist of an aqueous solution of ammonia containing for 75 example about 30 grams of ammonia per liter. Initially a conducting salt may be added to the anolyte, but the ammonium chloride formed during operation is sufficient to maintain the conductivity. In order to prevent the formation of 80 nitrogen trichloride which is very explosive, strong ammonia (specific gravity 0.880) should be added at intervals to the anolyte.

In practice it is found that good deposits may be obtained with catholytes containing as much 85 as about 30 grams per liter ammonium chloride. Any tendency of the concentration to increase too much may be remedied by increasing the rate of evacuation of the anolyte.

A system by means of which the catholyte may be fortified without interruption of the process is illustrated by way of example in the accompanying drawing. In this drawing the reference character 1 represents the anolyte chamber, 2 the catholyte chamber, and 3 the diaphragm. The catholyte is continuously drawn off by means of a siphon 4 which serves to maintain the level of the liquid in the catholyte chamber. The siphon delivers to a vessel 5 in which palladosammine chloride is dissolved. The solution passes to a 100 filter 6 and is then pumped to a feed vessel 7 and supplies the catholyte chamber 2. The catholyte may also be agitated in the actual plating cell as well as continuously circulated.

The deposits of palladium obtained by this 105 process are bright up to a thickness of about 0.00002 inch, but thicker deposits are somewhat milky, although they are adherent and suitable for buffing or other finishing operations.

The current density required to give the best 110

results varies with the other conditions, including the concentration of the metal salts and the temperature. As an example in palladium plating with a bath containing 15 grams of palladium per liter as tetrammine chloride the most suitable current densities at the specified temperatures were as follows:—

| 10 | Temperature of catholyte | Current density amps. per dm <sup>2</sup> |
|----|--------------------------|-------------------------------------------|
|    | 3° C.                    | 0.1 to 0.5                                |
|    | 20° C.                   | 0.5 to 1.0                                |
|    | 40° C.                   | 1.0 to 1.5                                |
| 15 | 70° C.                   | 2.0                                       |

15 The deposits at lower temperatures were brighter than those at high temperatures.

20 The catholyte may be formed by dissolving salts of palladium in ammonia either before use or in the catholyte. Thus, an ammoniacal solution of palladosammne chloride  $Pd(NH_3)_2Cl_2$  may be obtained by dissolving either palladium chloride or tetrammino-palladous chloride  $Pd(NH_3)_4Cl_2$ . In the same way other palladosammne salts, such as 25 the sulphate, carbonate, phosphate, bromide, nitrite, fluoride, acetate, tartrate, and citrate, may be dissolved in ammonia to form catholytes which give good adherent deposits. In the case of the chloride, ammonium pallado-chloride 30  $(NH_4)_2PdCl_4$  dissolved in aqueous ammonia yields the same electrolyte. Again, palladium may be deposited at about 50° C. from ammoniacal solutions of palladosammne oxalate. Ammoniacal 35 solutions of diammmino-dihydroxo-palladium or tetrammino-palladous hydroxide give particularly bright deposits.

As an example of the use of tetrammino-palladous hydroxide the following may be given:—

40 A catholyte containing about 20 grams palladium and about 5 grams free  $NH_3$ , both per liter, is prepared by adding excess of ammonia to an aqueous solution of dihydroxo-diammino-palladium made by a known method and is allowed to stand for twelve hours. The anolyte contains 45 20 grams ammonium sulphate and 100 cc. ammonia solution (specific gravity .880) per liter. Gelatin about .05 gram per liter is added to the catholyte. The ordinary porous pot diaphragm is used. At room temperature, 2 volts, and a current density of 0.3 amp. per dm<sup>2</sup>, bright adherent 50 deposits (up to .0001 inch thick) are obtained with a current efficiency of 94-97%.

55 As tetrammino-palladous hydroxide reacts with ammonium sulphate to form tetrammino-palladous sulphate, there is a tendency for the bath to lose its special character consequent on the diffusion of ammonium sulphate into the catholyte. Therefore the catholyte should be removed from the cell and stored in another vessel when plating is not in progress.

60 Such separate storing of the catholyte may advantageously be adopted in all cases, but is especially desirable in the case of tetrammino-palladous hydroxide.

65 The palladium amino compounds may also be formed by using organic amines such as pyridine and ethylenediamine instead of ammonia. Thus, an aqueous solution of palladium chloride and excess of pyridine may be used as the catholyte in conjunction with an aqueous solution of pyridine hydrochloride as the anolyte. Again, an aqueous solution of palladium chloride and excess of ethylenediamine hydrate may be used as the catholyte and an aqueous solution of ammonia and ammonium chloride at the anolyte.

The invention may be applied advantageously to certain other metals capable of forming metalammines soluble in aqueous ammonia and capable of yielding electrodeposits, namely rhodium, platinum, iridium, nickel, copper, silver, zinc, cadmium and cobalt. As is well known iron is not precipitated from solutions of its salts in the presence of tartrates and citrates and such solutions may be used for the electro-deposition of iron. These ammoniacal solutions may also be used as catholytes in this invention. Tin may also be deposited from ammoniacal catholytes containing tin chloride and ammonium tartrate. Furthermore, the invention may also be used for plating with or depositing alloys of the said metals, the catholyte in such a case consisting of a mixture of salts of the metals in question. Of course, not every alloy of the metals in question can be deposited in this way, because all the metals are not deposited with the same facility.

90 For the deposition of metals other than palladium the following salts which are capable of forming metalammine solutions in ammonia may be used:

95  $Ag_2SO_4$ ,  $ZnSO_4$ ,  $CdSO_4$ ,  $NiSO_4$ ,  $CoSO_4$ ,  $RhCl_3$ ,  $CuSO_4$  and  $Cu(NO_3)_2$ .

100 Platinum and iridium salts which may be used are:

105  $Pt(NH_3)_2Cl_2$ ,  $Pt(NH_3)_2(NO_2)_2$  and  $[Ir(NH_3)_5Cl]Cl_2$ .

110 The rhodium, platinum and iridium baths should be maintained at about 90° C. during the process in order to improve the current efficiency but the baths of the other metals may be worked either hot or cold.

115 Thus, as an example of the deposition of rhodium the following may be given: A solution containing about 7 grams rhodium as chloride and about 16 grams of urea per liter is boiled until a test portion gives no precipitate on adding excess of ammonia. During the boiling it may be found necessary to add a little hydrochloric acid to remove turbidity. Finally, excess of strong 120 ammonia solution (specific gravity .880) is added after which the solution is boiled. The anolyte contains 150 cc. of strong ammonia solution (specific gravity .880) and about 25 grams ammonium chloride per liter. At 70° C., 2 volts, and a current density of 0.3 amp. per dm<sup>2</sup> this bath gives 125 bright adherent deposits of rhodium with a current efficiency of 10%.

130 As an example of the deposition of iron the following may be mentioned: about 120 grams of ferrous ammonium sulphate crystals and about 80 grams of citric acid are dissolved in about 800 cc. water. After boiling and filtering, the filtrate is allowed to cool and then made ammoniacal by adding about 120 cc. of strong ammonia 135 solution (specific gravity .880); about 33 grams of ammonium sulphate are added and the volume made up to 1 liter. The anolyte contains about 40 grams ammonium sulphate and about 80 cc. of strong ammonia solution (specific gravity 140 .880) per liter.

140 At 60° C., 1.9 volts, a current density of 0.6 amp. per dm<sup>2</sup> and a plating time of 30 minutes a hard adherent deposit of iron is obtained on copper with a current efficiency of 30%.

145 As an example of the deposition of copper the following may be mentioned: A catholyte is taken containing about 12.5 grams per liter of copper as nitrate, about 20 grams per liter of ammonium nitrate, and a small excess of ammonia solution. 150

The anolyte contains about 50 grams of ammonium nitrate and 160 cc. of strong ammonia solution per liter.

At room temperature, 3.1 volts, a current density of 1 amp. per  $\text{dm}^2$  and a plating time of 30, minutes, an adherent deposit of copper is obtained on an aluminium cathode with a current efficiency of 64%.

In the case of copper the presence of ammonium salts is essential for satisfactory deposition.

As an example of the deposition of an alloy containing 90% palladium and 10% cobalt the following may be mentioned: A solution containing about 50 grams of cobalt sulphate crystals per liter and about 50 grams ammonium sulphate per liter is made ammoniacal and boiled with the addition of hydrogen peroxide for one hour. The solution is next cooled and filtered, and the filtrate mixed with an ammoniacal solution of tetrammino-palladous sulphate. The mixed solution containing about 14.4 grams palladium, about 1.4 grams cobalt, and about 3.4 grams ammonia, all per liter, is used as the catholyte with an anolyte containing about 40 grams ammonium sulphate and 120 cc. of ammonia solution (specific gravity .880) per liter. At room temperature, 3 volts, a current density of 1 amp. per square decimetre, and a plating time of 15 minutes, hard bright adherent deposits containing approximately 90% Pd, 10% Co are obtained on silver and copper cathodes with a current efficiency of 90%.

As an example of the deposition of a base metal alloy the following may be mentioned: Sufficient tartaric acid is added to a solution of ferrous ammonium sulphate to prevent the formation of a precipitate on making the solution ammoniacal. This solution is mixed with an ammoniacal solution of nickel sulphate to give a catholyte containing about 11 grams of iron, about 6 grams of nickel, about 40 grams of tartaric acid and 11 grams of free  $\text{NH}_3$  per liter. About 20 grams of ammonium sulphate per liter is added as conducting salt. The anolyte contains about 50 grams of ammonium sulphate and 150 cc. of strong ammonia solution (specific gravity .880) per liter. At room temperature, 2.5 volts, a current density of 0.4 amp. per  $\text{dm}^2$  and a plating time of 1 hour an alloy containing 70% nickel and 30% iron is deposited with a current efficiency of 59%.

At a temperature of 60° C. an alloy rich in iron (containing 80% Fe.) is obtained from the same electrolyte.

In certain cases addition agents may be added to the plating bath; thus for example the addition of 1% of ethylenediamine hydrate renders palladium deposits less milky, while urea serves to increase the current efficiency in the deposition of rhodium. Again, the addition of a small quantity of gelatin, of the order of about 0.05 gram per liter, to a tetrammino-palladous hydroxide catholyte gives bright fine-grained plates.

The preferred diaphragm consists of a porous pot of the same porosity and material as those used in Leclanché cells, but of course other porous materials may be used provided they are not attacked by the electrolyte, e. g. alundum and porous hard rubber are both suitable. The diaphragm may consists of a porous pot surrounding either the anode or the cathode or it may be

a porous partition (or partitions) separating the anolyte from the catholyte compartment (or compartments).

The anode may consists for example of lead, platinum, palladium or graphite.

The selection of the cathode metal will be determined by the metal which is to be deposited upon it. When used as the cathode for palladium plating copper, silver, palladium, lead, tin, "nickel-silver", brass and pewter among others, all lead to the formation of good adherent deposits and other metals such as nickel and iron may be plated after preliminary plating or coating with other metals such as copper and tin. In addition to the usual cathode metals used for electro-deposition it has been found that aluminium can be plated satisfactorily with copper, possibly because an ammoniacal electrolyte has less tendency to attack aluminium than the acid or alkaline electrolytes used in other plating processes.

Generally the cathodes will be stationary but moving cathodes may also be used in suitable cases.

As mentioned above, the invention is applicable to the electrolytic reduction of metals from their salts, such for example as the electrolytic recovery of silver from silver chloride or of palladium from palladosammie chloride. In such a case, of course, a cathode is preferably used from which the deposit may be easily stripped. For example, a carbon cathode may be used for silver, while in particular cases metal cathodes on which only flaky deposits are obtained in plating may advantageously be used in the reduction of metal salts.

I claim:—

1. A process for the electrodeposition of a metal or alloy which comprises establishing a porous pot diaphragm cell containing an ammoniacal anolyte substantially free from a metal compound, an insoluble anode, and a catholyte containing an ammoniacal solution of a metal to be electro-deposited; making an article to be plated a cathode in said cell; and passing a current through said cell to cause the electrodeposition on said article of metal from said ammoniacal catholyte.

2. A process for the electrodeposition of palladium which comprises establishing a porous pot diaphragm cell containing an anolyte of the group consisting of ammonia, organic amine and the like, an insoluble anode and a catholyte containing an ammoniacal solution of a palladium ammino compound; making an article to be plated a cathode in said cell; and passing a current through said cell to cause the electrodeposition in said article of palladium from said ammoniacal catholyte.

3. A process for the electrodeposition of palladium which comprises establishing a porous pot diaphragm cell containing an anolyte of the group consisting of ammonia, organic amine and the like, an insoluble anode and a catholyte containing an ammoniacal solution of palladosammie chloride; making an article to be plated a cathode in said cell; and passing a current through said cell to cause the electrodeposition in said article of palladium from said ammoniacal catholyte.

RALPH HALL ATKINSON.